

## 1

3,274,312

PROCESS FOR PREPARING DYE-RECEPTIVE  
SHAPED ARTICLES

Mario Compostella, Emanuele Del Mauro, and Giovanni Latella, Terni, Italy, assignors to Montecatini Società Generale per l'Industria Mineraria e Chimica, Milan, Italy  
No Drawing. Filed Dec. 17, 1962, Ser. No. 244,943  
Claims priority, application Italy, Dec. 21, 1961,  
22,809/61  
7 Claims. (Cl. 264—78)

The present invention relates to a process for preparing dye-receptive shaped articles such as textile fibers, films, sheets, tapes, etc., from alpha-olefin polymers.

In the applicant's U.S. patent applications Ser. No. 30,732, now abandoned, No. 124,346 and No. 212,119 there has been described a process for preparing basic nitrogen polycondensates by reacting (in the presence or absence of solvents and condensing agents) one or more primary  $C_3$ — $C_{30}$  or secondary  $C_4$ — $C_{60}$  aliphatic amines with epichlorohydrin, this first condensation being followed by a further condensation with one or more aliphatic, aromatic or heterocyclic-bis secondary diamines.

The preparation of shaped articles including textile fibers from mixes containing these polycondensates and of polyolefins prepared with the aid of stereospecific catalysts (see, for example, Italian Patent No. 526,101), more particularly polypropylene has also been described in the above applications.

Processes used for obtaining, for example, textile fibers, in general, comprise:

(1) Mixing the polycondensate (for example, 1—25% with respect to the total mix) with the polyolefin, employing any conventional known procedure;

(2) Granulating the mix obtained according to (1), in a screw device at temperatures of 170—300° C., in order to render the mix suitable for feeding into spinning devices; (it being known that the use of rough powdered mixtures, in fact, make the feeding operation irregular and therefore detrimentally affects the spinning step);

(3) The extrusion of the resulting granulate in a melt spinning device through spinnerets having holes with a length/diameter ratio preferably higher than 1, and winding the spinning filament;

(4) Stretching and spinning the filaments obtained in (3).

Various polycondensates, however, when they are subjected to the drastic thermal treatment needed for the granulation and spinning (stages 2 and 3 above) are altered thereby exhibiting a decrease in their molecular weight and a certain discoloration.

It has been now surprisingly found according to the present invention, that the thermal decomposition of dyeable basic nitrogen polycondensates can be avoided by eliminating the mix granulation stage, and, by sintering the polycondensate-polyolefin mix at temperatures between 20° and 170° C.

By carrying out this procedure, it is possible to obtain the mixes in the form of granules which can be fed to the spinning screws in a regular and homogeneous manner and which do not easily disintegrate.

In order to produce these sintered granules, any suitable continuous or discontinuous apparatus capable of supplying heat may be employed for the sintering step.

In the preparation of dyeable textile fibers from crystalline polyolefins, such as polypropylene containing predominant amounts (more than 50%) of isotactic macromolecules, it is convenient to prepare a mix rich in the basic nitrogen polycondensate, and then sinter this mix. Subsequently the polycondensate-rich granules are extruded or spun after adding thereto the amount of granular

## 2

polyolefin needed to achieve the desired amount of polycondensates in the textile fibers.

According to the present invention, 1—50% of polycondensate may be mixed with 50—99% of polyolefin.

The method of the present invention, more particularly, may be applied to mixes of polyolefins and basic nitrogen polycondensates obtained by reacting (in the presence or absence of solvents and condensing agents) (1) epichlorohydrin, (2) one or more primary  $C_3$ — $C_{30}$  or secondary  $C_4$ — $C_{60}$  aliphatic amines and then subjecting the condensation product to a further condensation with one or more aliphatic, aromatic or heterocyclic secondary diamines. These condensates show generally a softening point under 120° C., an intrinsic viscosity (determined in a 1% isopropanol solution) of 0.05—0.5 and a nitrogen content up to 35%.

Mixes of polypropylene with polycondensates of octadecylamine, epichlorohydrin and piperazine are of particular interest.

The shaped articles such as fibers are then prepared by extruding the granules sintered according to the invention. The mixes to be extruded contain polyolefins, from 1 to 25% by weight of the nitrogen polycondensate and, if desired, 0.1 to 5% of a "solid dispersing agent" for dispersing the nitrogen condensate in the molten mass. Suitable solid dispersing agents include: cetyl and stearyl alcohols, stearic acid, benzoin, furoin, vinyl stearate, mono-, di- or tristearic esters of glycerol, monoethanolamine stearate, stearic amide,  $C_6$  to  $C_{30}$  aliphatic amines, condensation products of ethylene oxide with alcohols, amines or phenols, polystearamide, polyacrylic acid, polystyrene, styrene copolymers, terpene polymers, etc.

The sintering and spinning operations according to the present invention may be conveniently carried out under oxygen-free nitrogen.

The fibers produced may be in the form of mono- or pluro-filaments and can be employed for preparing continuous fibers or staples or for preparing either bulky yarns or staples.

The mono- or pluro-filaments prepared according to the present invention can be subjected to treatments for the water-insolubilization of the basic nitrogen compound. Particularly useful for this purpose are the treatments with formaldehyde, diisocyanates, diepoxy compounds or various cross-linking agents such as divinyl benzene or the like. These treatments may be carried out either before or after stretching.

The stretching is preferably executed using ratios between 1:2 and 1:10 at temperatures between 80° and 150° C. in stretching devices heated with hot air, steam or similar fluids.

The fibers thus obtained can be dyed with acid dyes or with plasto-soluble dyes. They also exhibit a good affinity for basic and vat dyestuffs.

The sintered granules prepared according to the present invention are also suitable for extrusion into films, tapes and various other shaped articles.

The present invention is applicable to polyolefins, particularly polyolefins prepared by the stereospecific polymerization of alpha-olefins of the formula



wherein R is a hydrocarbon radical. Stereospecific catalysts such as those disclosed by Natta et al. or shown in Italian Patent 526,101, are examples of suitable catalysts.

Shaped articles, especially fibers obtained from polypropylene containing predominant amounts (more than 50%) of isotactic macromolecules are of particular interest.

The following examples are given to illustrate the present invention without limiting its scope.

All parts and proportions are by weight unless otherwise indicated.

The residue of the heptane extraction is an indication of the presence of isotactic macromolecules.

*Example 1*

A mix is prepared from:

(1) 100 kg. of polypropylene prepared with the aid of stereospecific catalysts having an intrinsic viscosity  $[\eta]$  of 1.45 (determined in tetrahydronaphthalene at 135° C.), a residue after heptane extraction of 96% and an ash content of 0.01%, and

(2) 5 kg. of a polycondensate prepared by reaction of 0.3 mol of n-octadecylamine with 1.3 mols of epichlorohydrin and 1 mole of piperazine.

The mix is then sintered in a machine for preparing tablets. The residence time of the mix in the sintering machine is 1 second, and this device reaches a temperature of 90° C.

The sintered granules are then spun in a melt spinning device under the following conditions:

Screw temperature, ° C. ----- 250  
Head temperature, ° C. ----- 260  
Spinneret temperature, ° C. ----- 260

Spinneret type, 192 holes with a diameter of 0.8 mm. and a height of 16 mm.

Max pressure (kg./cm.<sup>2</sup>) ----- 100  
Winding speed (m./min.) ----- 500

The yarns prepared as described have a clear color; and their intrinsic viscosity amounts to 90% of the initial value.

These yarns, after stretching at 130° C. in the presence of steam with a stretching ratio of 1:6 have the following serimetical characteristics:

Tenacity, g./den. ----- 6  
Elongation, percent ----- 20

Immediately after stretching, the yarn is wetted with a 5% aqueous ethylene glycol diglycidylether solution and then dried.

Upon dyeing these fibers colors, having good intensity and fastness are obtained with the folowing dyes:

Solid yellow 2G ----- Acid dye.  
Wool red B ----- Acid dye.  
Alizarine blue ACF ----- Acid dye.  
Acid black JVS ----- Acid dye.  
Lanasyn red 2GL ----- Metallized dye.  
Setacyl yellow 3G ----- Plastosoluble dye.  
Cibacet scarlet BR ----- Plastosoluble dye.  
Acetoquinone blue RHO ----- Plastosoluble dye.

*Example 2*

A mix is prepared from:

(1) 100 kg. of polypropylene obtained with the aid of stereospecific catalysts and having an intrinsic viscosity  $[\eta]$  of 1.60 (determined in tetrahydronaphthalene at 135° C.), a residue after heptane extraction of 94% and an ash content of 0.010%, and

(2) 5 kg. of the polycondensate prepared by the reaction of 5 mols of n-octadecylamine with 1.5 mols of epichlorohydrin and 1 mole of piperazine.

The mix is then sintered in a device for the preparation of tablets. The residence time of the mix in the sinterization device is 1 second and the mix reaches a temperature of 100° C.

The sintered granules are spun in a melt spinning device under the following conditions:

Screw temperature, ° C. ----- 260  
Head temperature, ° C. ----- 265  
Spinneret temperature, ° C. ----- 265  
Spinneret type, mm. ----- 198 x 0.8 x 16  
Maximum pressure, kg./cm.<sup>2</sup>. ----- 100  
Winding speed, m./min. ----- 500

The fibers thus prepared have a clear color and their residual intrinsic viscosity amounts to 85% of the initial value.

The fibers, after being stretched at 130° C. in the presence of steam with a stretching ratio of 1:5, exhibit the following serimetric characteristics:

Tenacity, g./den. ----- 6.5  
Elongation, percent ----- 22

Immediately after stretching, the fiber is wetted with a 5% aqueous solution of ethylene glycol diglycidyl ether and is then dried.

Colors having good intensity and fastness are obtained upon dyeing these fibers with the following dyes:

15 Solid yellow 2G ----- Acid dye.  
Wool red B ----- Acid dye.  
Alizarine blue ACF ----- Acid dye.  
Acid black JVS ----- Acid dye.  
Lanasyn red 2GL ----- Metallized dye.  
Setacyl yellow 3G ----- Plastosoluble dye.  
Cibacet scarlet BR ----- Plastosoluble dye.  
Acetoquinone blue ----- Plastosoluble dye.

*Example 3*

25 A mix is prepared from:

(1) 100 kg. of polypropylene prepared with the aid of stereospecific catalysts and having an intrinsic viscosity of 1.3 (determined in tetrahydronaphthalene at 135° C.), a residue after heptane extraction of 95% and an ash content of 0.029, and

(2) 5 kg. of a polycondensate prepared by reaction of 0.4 mol of n-dodecylamine with 1.4 mols of epichlorohydrin and 1 mol of piperazine.

The mixture is then sintered in a device for the preparation of pellets using a residence time in the sintering device of 1 sec. The mix is heated to a temperature of 80° C. in this device.

The centered granules are spun in a melt spinning device under the following conditions:

40 Screw temperature, ° C. ----- 240  
Head temperature, ° C. ----- 245  
Spinneret temperature, ° C. ----- 245  
Spinneret type ----- 198/0.8 x 16.  
Max. pressure, kg./cm.<sup>2</sup> ----- 100  
45 Winding speed, m./minute. ----- 500

The fibers so obtained are stretched at 130° C. in the presence of steam while employing a stretching ratio of 1:5. The fibers exhibit the following serimetric characteristics:

50 Tenacity, g./den. ----- 5.5  
Elongation, percent ----- 18

Immediately after stretching, the fibers are wetted with a 25% aqueous ethylene glycol diglycidyl ether solution and dried.

Colors having a good intensity and fastness are obtained upon dyeing the fibers with the following dyes:

55 Solid yellow 2G ----- Acid dye.  
Alizarine blue ACF ----- Acid dye.  
Acid black IVS ----- Acid dye.  
Lanasyn red 2GL ----- Metallized dye.  
Setacyl yellow 3G ----- Plastosoluble dye.  
Cibacet scarlet BR ----- Plastosoluble dye.  
65 Acetoquinone blue RHO ----- Plastosoluble dye.

Many variations and modifications may, of course, be employed without departing from the scope and spirit of the present invention.

70 Having thus described the invention, what it is desired to secure and claim by Letters Patent is:

1. In the process for preparing dye-receptive shaped articles by extruding a mix containing (1) an olefin polymer and (2) a basic nitrogen polycondensate, obtained from (a) at least one amine selected from the

group consisting of primary aliphatic amines containing 3-30 carbon atoms and secondary aliphatic amines containing 4-60 carbon atoms, (b) epichlorohydrin and (c) at least one member selected from the group consisting of aliphatic, aromatic and heterocyclic-bis secondary diamines, and stretching said shaped articles, the improvement which comprises transforming said mix into granules by sintering at a temperature of from 80° C. to about 170° C. before said extrusion step.

2. The process according to claim 1, wherein the mix which is sintered is rich in the nitrogen polycondensates and before extrusion thereof additional amounts of olefin polymer are added to said mix in order to obtain the desired proportions between the polycondensate and the olefin polymer.

3. The process according to claim 1, wherein from 0.1 to 5%, based on the total weight of the mix, of a solid dispersing agent for the nitrogen polycondensate is also present in said mix.

4. The process according to claim 1, wherein the olefin polymer is polypropylene consisting predominantly of isotactic macromolecules.

5. The process according to claim 1, wherein the basic nitrogen polycondensate is prepared by reacting 1 mol of a compound from (a), 1 to 3 mols of epichlorohydrin

5

20

15

25

and 0.1 to 10 mols of a bis- secondary diamine from (c).

6. The process according to claim 1, wherein the amine of (a) is selected from the group consisting of n-dodecylamine, hexadecylamine, octadecylamine, dioctadecylamine, dioctylamine or salts thereof.

7. The process according to claim 1, wherein the secondary diamine of (c) is piperazine.

#### References Cited by the Examiner

##### UNITED STATES PATENTS

|           |         |                 |       |        |
|-----------|---------|-----------------|-------|--------|
| 2,945,010 | 7/1960  | Caldwell et al. | ----- | 264—78 |
| 3,013,998 | 12/1961 | Battaglioli     | ----- | 264—78 |
| 3,059,275 | 10/1962 | Vogt.           |       |        |
| 3,098,697 | 7/1963  | Cappuccio       | ----- | 264—78 |
| 3,151,928 | 10/1964 | Cappuccio       | ----- | 264—78 |

##### FOREIGN PATENTS

|           |        |         |
|-----------|--------|---------|
| 1,245,063 | 9/1960 | France. |
|-----------|--------|---------|

ALEXANDER H. BRODMERKEL, *Primary Examiner.*

MORRIS LIEBMAN, *Examiner.*

C. B. HAMBURG, K. W. VERNON, A. L. LEAVITT,  
B. SNYDER, *Assistant Examiners.*